

# UNITED STATES PATENT OFFICE.

FRANK LAKE WILSON AND SIDNEY ELLIOTT BRETHERTON, OF BERKELEY,  
CALIFORNIA.

## PROCESS FOR PRECIPITATION OF ZINC.

1,083,785.

Specification of Letters Patent.

Patented Jan. 6, 1914.

No Drawing.

Application filed January 28, 1913. Serial No. 744,654.

To all whom it may concern:

Be it known that we, FRANK L. WILSON and SIDNEY E. BRETHERTON, citizens of the United States, and residents of Berkeley, in the county of Alameda and State of California, have invented a new and Improved Process for Precipitation of Zinc, of which the following is a full, clear, and exact description.

10 The purpose of this invention is to obtain a constant precipitation of metallic zinc from an electrolytic bath and obviate the necessity of installing reduction furnaces for the production of the same.

15 To carry out the above outlined object, we maintain the concentration of zinc ions in the electrolyte constant, and we obtain this by the addition of a zinc-containing substance to the electrolytic bath.

20 Our process is especially intended for the continuous precipitation of metallic zinc from either a hot or cold bath of electrolyte of zinc sulfate ( $ZnSO_4$ ) or zinc chlorid ( $ZnCl_2$ ). The solution of zinc sulfate or chlorid of a proper strength is introduced 25 into a vat provided with anodes and cathodes, the solution forming electrical connection between these electrical poles, so that when the electric current is passed the electrolyte, hot or cold, under the action of the electric current decomposes, and the metallic zinc precipitates at the cathode while the radical ions of the acid are evolved 30 at the anode. Thus the ionic strength of the

35 solution in zinc decreases while the acid in the solution becomes concentrate. To keep the ionic strength of zinc constant and prevent the concentration of the acid in the electrolytic bath, we add to this solution intermittently or continuously zinc oxid ( $ZnO$ ) 40 or zinc carbonate ( $ZnCO_3$ ) or both together, pure or contaminated, while the bath is under the action of electric current. The addition of these substances to a bath of either 45 zinc chlorid or zinc sulfate may be expressed by the reaction as follows:—



50 The above equations show the reaction of the hydrochloric acid and the sulfuric acid present in the respective baths due to the precipitation of metallic zinc and which is

55 prevented from concentration by the addition of the zinc oxid or zinc carbonate, or both together. The reaction for both together in a bath is not shown, as it can be easily figured out from the two reactions shown for zinc oxid and zinc carbonate.

60 We also add to the electrolyte ammonium carbonate  $(NH_4)_2CO_3$  to form in the bath ammonium sulfate  $(NH_4)SO_4$  or ammonium chlorid, each of which causes a better and more uniform precipitation of metallic zinc at the cathodes, from an electrolyte 65 of zinc sulfate or chlorid, respectively; that is, it adds to the transmission of the ions and acts as a catalytic agent. The addition of ammonium carbonate can be made directly, or the zinc oxid and zinc carbonate added 70 are contaminated with ammonia ( $NH_3$ ) and free carbon dioxid ( $CO_2$ ). When pure zinc oxid or zinc carbonate is used the addition of ammonium carbonate can be made direct to the bath. The reaction is as follows:— 75



80 The above represents the reactions occurring when the zinc carbonate and the zinc oxid are contaminated with ammonia and carbon dioxid. These gases cling more or less to the precipitate and unless thoroughly dried will remain and pass into the electrolyte. 85

When the ammonium sulfate or chlorid becomes too concentrated it proves a detriment to the precipitation of the metallic zinc. The fouled solution is then passed to 90 proper stills where the ammonium is recovered, lime being used to free the ammonia.



95 A similar equation can be written for ammonium chlorid. Thus, the ammonium can be used over and over again. The carbon dioxid formed in the reaction when using zinc carbonate for the electrolytic bath may be collected in any similar way and combined with the recovered ammonia to form ammonium carbonate, which can then be added to the electrolytic bath, or formed in the bath by contaminating the zinc oxid and carbonate with the recovered gases. 100

105 As the zinc carbonate is generally more

or less hydrated, another reaction may take place as shown below:



We find that the coefficient in the hydrated zinc carbonate is 3; that is, the formula for hydrated zinc carbonate may be written as  $ZnCO_3 \cdot 3H_2O_2$ . Other complete reactions, as shown before for zinc oxid and 10 zinc carbonate, can be similarly expressed with the hydrated zinc carbonate.

It can be easily seen that with our process, by the addition of a zinc oxid and zinc carbonate, the ionic strength of zinc in the 15 electrolytic bath is maintained constant. This permits a constant precipitation of metallic zinc by means of the electric current, and the addition of ammonia carbonate to the electrolyte makes the precipitation 20 more uniform.

While to all the reactions described ammonium carbonate was used, acid ammonium carbonate can as well be used for the same purpose, as it can be easily seen without 25 showing its reactions by means of equation.

Having thus described our invention, we claim as new and desire to secure by Letters Patent:

1. The process for the continuous precipitation of metallic zinc, which consists in forming a solution of zinc sulfate, then introducing said solution into a container provided with anodes and cathodes, said solution establishing electrical communication 30 between said anodes and cathodes, then passing the current therethrough thereby decomposing said solution, the zinc being deposited on the cathodes, and to said solution adding zinc carbonate to maintain the 35 strength of the solution substantially constant, and similarly adding to this solution ammonium carbonate to form an ammonium sulfate which acts as a catalytic agent in the electrolyte, and the deposit of the zinc on 40 the cathodes is more uniform due to its presence.

2. The process for the continuous precipitation of metallic zinc, which consists in forming a solution of zinc sulfate, then introducing said solution into a container provided with anodes and cathodes, said solution establishing electrical communication between said anodes and cathodes, then passing the current therethrough thereby decomposing said solution, the zinc being deposited on the cathodes, and to said solution adding hydrated zinc carbonate to maintain the strength of the solution substantially 50 constant, and similarly adding acid am-

monium carbonate to form an ammonium sulfate which acts as a catalytic agent in the electrolyte, and the deposit of the zinc on the cathodes is more uniform due to its presence.

3. The process for continuous precipitation 60 of metallic zinc, which consists in forming a solution of zinc sulfate, then introducing said solution into a container provided with anodes and cathodes, said solution establishing electrical communication between said 65 anodes and cathodes, then passing an electric current therethrough whereby said solution is decomposed, the zinc being deposited on the cathodes, and to the solution adding zinc carbonate to maintain the zinc 70 solution substantially constant, similarly adding to this solution ammonium carbonate to make the precipitation of metallic zinc on the cathodes more uniform, and removing the liberated carbon dioxid and the ammonium by proper means and using the same over again to form the ammonium carbonate.

4. In an electro-chemical process for the continuous precipitation of metallic zinc 85 from an electrolytic bath of zinc sulfate, a step consisting in adding zinc carbonate contaminated with ammonia and carbon dioxid to the electrolyte to maintain the ionic strength of the zinc in said bath substantially 90 constant and to make the precipitation of the zinc on the cathodes more uniform by the electric current.

5. In an electro-chemical process for the continuous precipitation of metallic zinc 95 from an electrolytic bath of the same, a step consisting in adding zinc carbonate contaminated with ammonia and carbon dioxid to the electrolyte to maintain the ionic strength of the bath substantially constant and to 100 make the precipitation of the zinc on the cathodes more uniform by the electric current.

6. In an electro-chemical process for the continuous precipitation of metallic zinc 105 from an electrolytic bath of the same, a step consisting in adding zinc carbonate and ammonium carbonate to form in the bath an ammonium salt which acts as a catalytic agent in the electrolyte.

In testimony whereof we have signed our names to this specification in the presence of two subscribing witnesses.

FRANK LAKE WILSON.

SIDNEY ELLIOTT BRETHERTON.

Witnesses:

FLORA HALL,  
A. E. LOWRIE.